

## [54] ASHLESS ANTI-RUST ADDITIVES

[75] Inventors: **Aart Strang; Bernard R. Talens**,  
both of Amsterdam, Netherlands[73] Assignee: **Shell Oil Company**, New York, N.Y.[22] Filed: **Aug. 28, 1970**[21] Appl. No.: **68,039**

## [30] Foreign Application Priority Data

Sept. 10, 1969 Great Britain.....44,633/69

[52] U.S. Cl. ....**252/57, 252/48.6, 252/396,**  
44/70, 44/76[51] Int. Cl. ....**C10m 1/20, C10m 1/38**[58] Field of Search .....**252/57, 396; 44/70**

## [56] References Cited

## UNITED STATES PATENTS

2,835,635 5/1958 Mayhew et al. ....**252/57**2,604,451 7/1952 Rocchini .....**252/51.5 A**  
2,682,489 8/1954 von Fuchs .....**252/56 D**

## FOREIGN PATENTS OR APPLICATIONS

809,198 2/1959 Great Britain.....**252/57***Primary Examiner*—Daniel E. Wyman*Assistant Examiner*—W. Cannon*Attorney*—Howard M. Flournoy and Glen R. Grunewald

## [57]

## ABSTRACT

Para hydrocarbyl-substituted phenol or thiophenol dicarboxylic acids as anti-rust and anti-corrosion additives to liquid hydrocarbon fuels and lubricants.

4 Claims, No Drawings

## ASHLESS ANTI-RUST ADDITIVES

## BACKGROUND OF THE INVENTION

Known anti-rust additives for oils may be divided functionally into two groups:

1. those which neutralize the acids present in the oil; and

2. those which form a thin layer on a metal surface, thus protecting it against the action of corrosive agents.

Additives of the first group usually contain metal atoms and they are quickly depleted and therefore must be applied in rather high concentrations. Particularly when these additives are incorporated in lubricant oils that are used as motor oils in internal combustion engines. The high concentration and metal content are disadvantageous because they form ash. Additives of the second group, which are less readily depleted, can be applied in lower concentrations. Moreover, they do not form ash.

## THE INVENTION

This invention relates to anti-rust additives of the second group which are hydrocarbyl substituted phenol or thiophenol dicarboxylic acids. These additives display excellent anti-rust properties and are non-ash forming. The invention therefore relates to liquid hydrocarbons containing aromatic dicarboxylic acids having the general formula:



wherein X is OH or SH, R is a straight or branched chain, cyclic or acyclic, alkyl, aryl or alkaryl hydrocarbyl group having from about six to 24 carbon atoms; and each R<sub>1</sub> may be hydrogen or a hydrocarbyl group having less than 24 carbon atoms. These acids have good solubility in hydrocarbon oils, are excellent rust inhibitors and show only a slight copper-lead corrosion.

The liquid hydrocarbons, such as fuels or lubricating oil compositions, contain a minor proportion of one or more of the aromatic dicarboxylic acids of the above formula. The present compounds may be utilized as anti-rust additives for mineral and synthetic lubricating oils which are employed as motor oils in internal combustion engines. Mineral oils that are generally paraffinic and/or naphthenic are preferred, although they may contain substantial proportions of aromatic hydrocarbons, a single neutral base or a mixture or blend of base stocks or a bright stock may be used as the base stock. Any suitable high-viscosity index or middle viscosity index base stock or mixtures thereof can be used. However, with the use of a suitable viscosity index (VI) improver oils of somewhat lower VI as for example 65 or less may also be used. The compounds according to the invention may also be utilized as anti-rust additives in distillate or residual hydrocarbon fuels and have been found especially effective when used in gasolines. The additives of this invention are useful in leaded or unleaded gasoline compositions.

In the additives of this invention, X is preferably a hydroxyl group. Especially suitable additives are 2-

hydroxybenzene-1,3-dicarboxylic acids in which both of the R<sub>1</sub> substituents are hydrogen atoms. R is preferably an aliphatic hydrocarbon group having more than 12 carbon atoms. For example, a preferred additive is 2-hydroxy-5-cetyl-benzene-1,3-dicarboxylic acid, 2-hydroxyl-5-lauryl-benzene-1,3-dicarboxylic acid, 2-hydroxy-5-stearyl-benzene, 1,3-dicarboxylic acid, 2-hydroxy-5-cetyl-benzene-1,3-dicarboxylic acid.

2-hydroxybenzene-1,3-dicarboxylic acids having an aliphatic hydrocarbon substituent attached to the benzene nucleus in para position relative to the hydroxyl group may be prepared by alkylation of phenol followed by phenation, carboxylation and hydrolysis. The presence of a hydrocarbon substituent attached to the benzene nucleus in para position relative to the hydroxyl group is an essential feature of the present invention, and the alkylation is therefore carried out with an alkylation agent for phenol that attacks the benzene nucleus preferentially in a position para to the hydroxyl group.

Examples of such agents are monoolefins, which are branched at one or both of the carbon atoms adjacent to the double bond, such as tetra-isobutene and higher polyisobutenes, or precursors of these olefins, such as monohydroxy alkanes in which the hydroxyl group is attached to a tertiary carbon atom or to a carbon atom that is in an alpha-position relative to a tertiary carbon atom in the molecule. Further examples of suitable alkylating agents are 1-methylcyclohexene and the product obtained by alkylation of ortho-cresol with cetene-1 followed by hydrogenation of the alkylate.

When the aromatic dicarboxylic acids according to the invention are used as anti-rust additives in lubricants or fuels, their concentrations can vary within wide limits. The additives are preferably added in an amount from about 0.01 to about 5.0 percent w, especially from 0.05 to 1.0 percent w.

In addition to the present acids, lubricants or fuel compositions can contain other additives. For example, if the acids are added to a lubricant, the latter may also contain anti-oxidants, extreme pressure agents, anti-wear agents, viscosity-index improvers, thickeners, dispersants, anti-foam agents and other substances known in the art to perform a particular function or functions provided they are otherwise compatible.

## EXAMPLE I

## 50 Preparation of 2-Hydroxy-5-cetylbenzene-1,3-dicarboxylic acid (Compound I)

A mixture of ortho- and para-cetylphenol obtained by alkylation of phenol with cetene-1 was subjected to phenation, carboxylation and hydrolysis. In this way a mixture of 2-hydroxy-5-cetylbenzene-1,3-dicarboxylic acid (from para-cetylphenol) and 4-hydroxy-5-cetylbenzene-1,3-dicarboxylic acid (from ortho-cetylphenol) was obtained. From this mixture the 2-hydroxy-5-cetylbenzene-1,3-dicarboxylic acid (Compound I) was isolated by chromatography.

## EXAMPLE II

To determine the anti-rust properties of compounds according to the invention in a lubricating oil, Compound I was compared with five commercial anti-rust additives (Compounds A-E) in a laboratory corrosion test. In this test the corrosion is measured continuously

by recording the change in the resistance of a standard iron wire (0.1 mm) immersed in an emulsion of a lubricating oil in which the anti-rust additive concerned has been incorporated. The lubricating oil emulsion is prepared by emulsifying an SAE oil containing 7.5 percent w of commercial viscosity index (VI) improver, 0.75 percent w of a commercial anti-oxidant and 1 percent w of a commercial anti-scuffing agent with 5 percent w of a synthetic water phase. The synthetic water phase which is representative of the water phase in an engine contains 0.6 N HCl, 0.3 N Al(NO<sub>3</sub>)<sub>3</sub> and 0.1 N (NH<sub>4</sub>)<sub>2</sub>SO<sub>4</sub>.

The test conditions of this laboratory corrosion test closely resemble but are much more severe than those prevailing in an ordinary engine.

The results of these tests are summarized in Table I.

Table I

| Compound | Composition                                    | Corrosion rate, mm/year<br>at a concentration of<br>0.1%w 0.5%w | 20 |
|----------|------------------------------------------------|-----------------------------------------------------------------|----|
| I        | 2-hydroxy-5-cetylbenzene-1,3-dicarboxylic acid | 0.05                                                            |    |
| A        | calcium naphtha sulphonate                     | 0.15(1%)                                                        |    |
| B        | phosphoric esters                              | 0.1 0.1                                                         |    |
| C        | superbasic magnesium salt                      | 0.1 <0.01                                                       |    |
| D        | tetrachlorophthalic acid                       | 0.3 1.2                                                         |    |
| E        | dodecetyl succinic acid                        | 0.5 0.4                                                         |    |
|          | Reference oil without anti-rust additives      | 0.5 - 0.7                                                       |    |

It may be seen from Table I that the additive of this invention even in very low concentrations is more effective as a rust inhibitor than other commercial preparations used for this purpose.

## EXAMPLE III

Since only compounds I, B and C were adequate as rust inhibitors in Example II. These compounds were tested to determine their corrosivity toward lead and copper, two common bearing materials. In the test 0.1 percent w of the indicated compound was added to the same reference oil under identical conditions and the corrosivity of each composition was measured as loss of weight of the copper and lead specimens immersed in the oil. The reference oil alone was of course substantially non-corrosive, but it was otherwise unsuitable because it was not rust inhibited.

The results of these tests are summarized in Table II.

Table II

| Compound                                     | Copper-lead corrosion<br>mg/cm <sup>2</sup> .h |       |
|----------------------------------------------|------------------------------------------------|-------|
|                                              | Copper                                         | Lead  |
| I                                            | 0.03                                           | 0.08  |
| B                                            | 0.006                                          | 1.10  |
| C                                            | 0.017                                          | 0.003 |
| Reference oil without<br>anti-rust additives | 0                                              | 0.01  |

## EXAMPLE IV

Since composition B proved too corrosive toward lead it was unsuitable and compositions I and C were further tested. The further tests involved employing oil 5 rust-inhibited with compositions I and C in a Ford-An-glia engine operated at constant speed (2,000 rpm) and constant power (6 bhp) for 24 hours, while the top cover of the engine was cooled to 4.5°C to promote condensation of the blow-by gases. The degree or rate 10 of corrosion in these tests was assessed by:

1. the loss in weight of the push rods;
2. the loss in weight of new mild-steel test plates in the top-cover area; and
3. the loss of weight of the dipstick.

The results of the motor tests are summarized in Table III.

Table III

| Composition<br>no.                           | Concentration<br>%w | Loss in weight, mg, of |              |          |
|----------------------------------------------|---------------------|------------------------|--------------|----------|
|                                              |                     | test<br>plates         | push<br>rods | dipstick |
| I                                            | 0.05                | 35                     | 15           | 6        |
| I                                            | 0.0                 | 28                     | 14           | 1        |
| C                                            | 0.025               | 91                     | 26           | 21       |
| C                                            | 0.5                 | 72                     | 14           | 0        |
| Reference oil without<br>anti-rust additives |                     | 134                    | 218          | 41       |

In addition to being more corrosive, composition C is an ashforming composition that has the above-mentioned adverse affects in lubricants.

From the foregoing it is evident that the ashless compositions of this invention are effective anti-rust additives for hydrocarbon liquids, and that they are non-corrosive. Other compositions of this invention produce equivalent, although not identical results when 35 incorporated into different hydrocarbon liquids.

We claim as our invention:

1. An ashless hydrocarbon lubricating oil composition containing a minor amount effective to inhibit rust of a hydrocarbyl-substituted aromatic dicarboxylic acid 40 having the general formula



wherein X is OH, R is an alkyl group of between more 50 than 12 and 24 carbon atoms, and each R<sub>1</sub> is hydrogen.

2. The composition of claim 1 wherein the lubricating oil is a mineral oil.

3. The composition of claim 2 wherein the dicarboxylic acid is 2-hydroxy-5-cetylbenzene-1,3-dicarboxylic acid.

4. The composition of claim 1 containing from about 55 0.01 to 5 percent w of the dicarboxylic acid.

\* \* \* \* \*